

## UNITED STATES PATENT OFFICE

2,553,449

## PROCESS FOR OBTAINING BY GALVANIC MEANS A COATING FOR PROTECTING MAGNESIUM FROM CORROSION

Herbert Manfred Freud, Nanterre, France

No Drawing. Application April 18, 1946, Serial No. 663,248. In France July 26, 1945

6 Claims. (Cl. 204—56)

1

In my copending application (on which Patent No. 2,463,483 issued March 1, 1949) Serial No. 314,349, filed January 17, 1940, I described a process for obtaining by galvanic means a coating for protecting magnesium from corrosion, such coating being produced by a galvanic process.

The preferred solution, which was used in that process contained the bi-valent ion  $Mn^{++}$  associated with an anion which does not attack the metal chemically, such as  $Cr_2O_7^{2-}$ .

In the process set forth in Ser. No. 314,349, several manganese salts such as the nitrates, the chlorides, the sulphates, were stated not to be capable of producing a good protective layer on magnesium, because they produce an attack on the metal.

The improved process which is the object of the present invention is related to this same technique of action by galvanic means as opposed to action by chemical means, and herein, as in Ser. 314,349, no electric current from outside is supplied.

One of the great advantages of protecting magnesium by galvanic means under the conditions of the present case (in addition to the improved resistance to corrosion) is that it is possible, in certain conditions, and in particular by the process which is the object of application Serial No. 314,349, to provide an excellent protective coating without producing a considerable change of dimensions, when treating calibrated parts.

Before starting the description of the process which is the object of the present invention and in order to make more apparent the importance of this fundamental distinction which exists between the action by chemical means and action by galvanic means, some indications will first of all be given concerning the phenomena which characterise the action by chemical means in the reactions relating to the treatment of magnesium.

The chemical attack of magnesium is generally manifested by one of the two following phenomena:

1. A progressive dissolution of a surface portion of the metal, without leaving any chemically produced covering occurs, and the amount of the metal so dissolved can be evaluated by the loss in weight of the metal during its immersion in the solution.

Thus, a plate of  $1 \text{ dm}^2$  (total surface area, on both sides) of an alloy of magnesium containing 1.8% of manganese was immersed in a solu-

tion containing 0.6% of  $Mn^{++}$  ion and 10% of  $CrO_3$  obtained by dissolving 100 gr. of  $CrO_3$  in 900 cc. of water and adding thereto 10 gr. of  $MnCO_3$ . This solution has a pH less than 1. It is difficult to accurately determine the pH of this solution by the scientific methods known at present, owing to the presence of a large proportion of  $CrO_3$ , the oxidizing power of which is considerable, but the pH is less than 1, measured by the glass electrode. Said plate weighed 9.125 gr. before it was introduced into the bath, and 8.941 gr. after remaining therein one hour. The loss of weight is therefore 0.184 gr. The decrease in thickness of the plate was more than  $2/100 \text{ mm}$ . (i. e. somewhat over 0.02 mm.).

2. Dissolution of a portion of the metal and the simultaneous coating of the metal with a layer of which the colour varies from yellow to mordoré (brownish crimson), brown or black. This layer is more or less adherent to the magnesium and, according to its thickness, is of greater or lesser weight which may to some extent counterbalance the thickness and weight of metal lost by solution.

25 Thus, a plate of  $1 \text{ dm}^2$  (total surface area, on both sides) of an alloy containing 1.8% of manganese was immersed for an hour in a solution containing 10% of  $Na_2CrO_4$  and 8% of  $KHSO_4$  ( $pH=5.7$ ). Said plate initially weighed 9.087 gr., and 9.039 gr. after remaining in the bath for one hour. During that treatment it became covered with a black film dotted with yellow spots. The apparent loss of weight was therefore only 0.048 gr.

30 But, when this black film was removed, by successive immersions in hot solutions of soda and of sodium hyposulphite ( $Na_2S_2O_3$  which is commonly called "hypo"), the plate weighed only 8.954 gr. The real loss of weight in the metal itself, is therefore 0.133 gr. or a decrease of thickness of the metal sheet of about 0.015 mm.

35 In the absence of ions other than  $Mn^{++}$  and  $Cr_2O_7^{2-}$  or  $CrO_4^{2-}$ , the chemical attack takes place only if the pH of the bath is very low, i. e. much below 2.5. In contradistinction, in the presence of ions such as  $SO_4^{2-}$ , the chemical attack takes place at a pH of nearly 6, or at any pH lower than this if the bath contains any considerable concentration of such ions.

40 My research work has enabled me to discover the conditions under which with baths in which the acid ion is composed principally of  $Cr_2O_7^{2-}$  or

$\text{CrO}_4^-$  the galvanic action takes place without there being a chemical attack on the magnesium, and on the other hand to discover that, as an exception to the general rule, mentioned in application Ser. No. 314,349, and the accuracy of which has been practically confirmed by practice, that the presence of sulphates, chlorides or nitrates produced an attack on the metal, the chemical action did not occur if the acid ion concentration is maintained within certain limits hereinafter defined.

Consequently, the object of the present invention is a process for protecting, by galvanic action, metal objects, by means of a bath mainly containing as anion one of the  $\text{Cr}_2\text{O}_7^{2-}$  or  $\text{CrO}_4^{2-}$  ions and which consists in operating with certain conditions of pH and of concentration which are defined hereinafter:

1. According to the invention, when the operation is effected in the absence of ions other than  $\text{Mn}^{++}$  and  $\text{Cr}_2\text{O}_7^{2-}$  or  $\text{CrO}_4^{2-}$  the pH should be maintained, in order that the galvanic action may be effected in satisfactory conditions, between 2.5 and 3.5 for a fresh bath. It is advisable in practice to keep the pH at about 3.

I have found that at a pH below 2.5 and at a pH much above 3.5, the treatment is too slow for the application of the process to be satisfactory industrially.

2. The operation may be effected in the presence of very small quantities of an active mineral acid, which will be obtained by the addition of ions such as  $\text{SO}_4^{2-}$ ,  $\text{NO}_3^-$ ,  $\text{PO}_4^{3-}$ , either in the form of acids, or in the form of salts. In particular  $\text{SO}_4^{2-}$  gives good results whether it is introduced in the form of sulphuric acid or of sulphates, or again in the form of sulphonated organic acids. Under these conditions (i. e. with a very small amount of  $\text{H}_2\text{SO}_4$  added), an electrolyte having a pH up to 3.95 may be satisfactory for use, (see table below).

For this addition of these acid ions not to produce any chemical attack, the bath must be such that the potential at the magnesium electrode formed by the object to be treated is less than 1.1 volts.

The concentration of such active mineral acid ions should be less than 0.5% and in particular it should be less than the figures:

$$\begin{aligned}\text{SO}_4^{2-} &< 0.1\% \\ \text{NO}_3^- &< 0.5\% \\ \text{PO}_4^{3-} &< 0.2\%\end{aligned}$$

The pH should be higher than 2.5. The upper limit of 3.5 is mentioned as being inadvisable to exceed owing to the slowness of the galvanic action, when the  $\text{Mn}^{++}$  and  $\text{Cr}_2\text{O}_7^{2-}$  or  $\text{CrO}_4^{2-}$  ions alone are present in the electrolyte. But this limit may be considerably exceeded in the presence of sulphuric, nitric or phosphoric acids or their salts since the presence of small quantities of the acid radicals of these acids increases the oxidizing power of the bath.

The table given hereinafter, which gives, for a series of proportions of constituents, the value of the pH and that of the potential at the magnesium electrode, relatively to the hydrogen electrode, illustrates the fact that according to the proportions, either a chemical attack occurs (which is very undesirable), or, on the contrary, only a galvanic action.

In practice, for these measurements, in view of the present difficulty in operating with hydrogen electrodes, I have used as a reference electrode a calomel electrode with saturated potas-

sium chloride, subtracting from this value 0.25 volt in order to bring the values observed down to those which would have been given by direct observation with the hydrogen electrode.

| Item      | Bath composition (per liter)                          | pH   | E    |                  |
|-----------|-------------------------------------------------------|------|------|------------------|
| a.....    | 10 grs. $\text{CrO}_3$ and 5.8 grs. $\text{MnCO}_3$ . | 3.8  | 0.90 |                  |
| b.....    | Item a plus 0.1 cc. $\text{H}_2\text{SO}_4$ .         | 3.2  | 1.02 |                  |
| c.....    | Item a plus 0.3 cc. $\text{H}_2\text{SO}_4$ .         | 2.2  | 1.15 | chemical attack. |
| d.....    | 100 grs. $\text{CrO}_3$ and 58 grs. $\text{MnCO}_3$ . | 2.   | 1.21 | Do.              |
| e.....    | Item d plus 0.1 cc. $\text{H}_2\text{SO}_4$ .         | 1.86 | 1.32 | Do.              |
| f.....    | 10 grs. $\text{CrO}_3$ and 6 grs. $\text{MnCO}_3$ .   | 4.25 | 0.67 |                  |
| 15 g..... | Item f plus 0.1 cc. $\text{H}_2\text{SO}_4$ .         | 3.8  | 0.89 |                  |
| h.....    | 100 grs. $\text{CrO}_3$ and 60 grs. $\text{MnCO}_3$ . | 2.05 | 1.16 | Do.              |
| i.....    | Item h plus 0.1 cc. $\text{H}_2\text{SO}_4$ .         | 1.95 | 1.24 | Do.              |
| j.....    | 10 grs. $\text{CrO}_3$ and 6.5 grs. $\text{MnCO}_3$ . | 4.5  | 0.61 |                  |
| 20 k..... | Item j plus 0.2 cc. $\text{H}_2\text{SO}_4$ .         | 3.95 | 0.84 |                  |
| l.....    | 100 grs. $\text{CrO}_3$ and 65 grs. $\text{MnCO}_3$ . | 3.95 | 0.87 |                  |
| m.....    | Item l plus 0.2 cc. $\text{H}_2\text{SO}_4$ .         | 3.8  | 0.95 |                  |
| n.....    | Item l plus 1.2 cc. $\text{H}_2\text{SO}_4$ .         | 3.2  | 1.18 | Do.              |

The figures in the column marked E, in the above table show the computed potential of the magnesium electrode relatively to the hydrogen electrode.

25 25. If, instead of the  $\text{SO}_4^{2-}$  ion,  $\text{NO}_3^-$  and  $\text{PO}_4^{3-}$  ions were used, a similar table would be obtained. In the latter cases also chemical attack occurs when the potential at the magnesium electrode relative to the hydrogen electrode, is greater than 1.1 volts.

30 30. It should be noted that the small quantities of  $\text{NO}_3^-$  ions carried along as a result of the usual depolarising operations of carbons by means of nitric acid, followed by a thorough washing, do not substantially alter the limits given in either of the above mentioned cases. However, it is possible, on the contrary, to limit the washing so as to allow sufficient  $\text{NO}_3^-$  ions to remain for the acidity to be maintained within the above mentioned limits.

35 35. By way of examples, given for the sole purpose of facilitating the comprehension of the present description, it is possible to proceed as follows:

45. Example I

A solution is prepared by dissolving in 1 litre of water, 10 gr. of  $\text{CrO}_3$ , and 5.8 gr. of manganese carbonate are then added, and then 0.1 cc. of sulphuric acid. The pH of this bath is 3.2.

50 50. A plate of an area of  $1 \text{ dm}^2$  (total surface area, on both sides) of magnesium alloy containing 1.8% of manganese is immersed therein. The potential relatively to the hydrogen electrode is 1.02 volts. The plate weighs 8.984 gr. before it is immersed in the bath and 8.975 gr. after an immersion of 1 hour. There is no yellow or brown film formed on the plate. The loss of weight is therefore only 0.009 gr., or a decrease of thickness of the sheet of 0.001 mm. No appreciable chemical attack has therefore occurred.

55 55. If this plate is electrically connected to a carbon counter-electrode, a cell is obtained having an electromotive force of 1.9 volts. By closing the circuit, a current of 70 milliamps flows, at a potential of 0.9 volts.

60 60. After a suitable period of treatment, (e. g. one hour), this piece is withdrawn, washed and dried; it is covered with a dark grey coating, and weighs 9.001 gr. The coating formed therefore weighs 0.026 gr.

Example II

75 75. Into a solution prepared from 1 litre of water, 10 gr. of  $\text{CrO}_3$  and 6 gr. of  $\text{MnCO}_3$ , there has been carried (from the depolarisation of the

carbons in nitric acid) 0.5 gr. of  $\text{HNO}_3$ . The bath accordingly contains about 0.05%  $\text{HNO}_3$ . The pH of this bath is 3.3.

A plate of an area of 1  $\text{dm}^2$  (total surface area, on both sides) of a magnesium alloy containing 1.8% of manganese is immersed therein. The potential relatively to the hydrogen electrode is 0.9 volt. The plate weighs 9.016 gr. before immersion in the bath and 9.016 gr. after an immersion of one hour. There is therefore no chemical attack whatever.

If carbon counter-electrode is placed opposite this magnesium alloy plate, a cell is obtained having an electromotive force (in open circuit) of 1.78 volts. By closing the circuit, a current of 55 millamps flows at 0.85 volt.

After a suitable period of treatment (1 hour, for example), the piece is withdrawn, washed and dried. It is covered with a brown film and weighs 9.032 gr. The coating formed therefore weighs 0.016 gr.

### Example III

To a solution prepared by dissolving 100 gr. of chromic acid in 1 litre of water, are added 66 gr. of  $\text{MnCO}_3$ , 1.2 gr. of  $\text{MnSO}_4$  corresponding to 0.75 gr. of  $\text{SO}_4$  ion. The pH of the bath is 3.7. A plate made of magnesium alloy containing 2.7% of aluminium, 0.3% of manganese and 1% of zinc and having an area of 1.2  $\text{dm}^2$  (total, for both sides of plate) is immersed therein.

The potential of the Mg relatively to the hydrogen electrode is 0.98 volts. When the circuit is open the electromotive force between the Mg and a counter-electrode of carbon is 1.88 volts. By closing the circuit a current of 60 millamps flows at 0.90 volts. After a period of treatment of 3/4 hour, the piece is withdrawn, washed and dried.

The durations of the galvanic action mentioned hereinbefore may vary according to the thickness of the protective layer to be obtained. If the duration is too short, the layer is insufficiently thick; if it is too long, the layer is too thick but a decrease of adherence is observed and it may have a tendency to scale.

The operations are carried out at temperatures of from 0° to 50° C. and preferably at room temperature.

### I claim:

1. A process of providing a protective coating upon a metallic article composed substantially entirely of magnesium and magnesium base alloy, by galvanic action, which comprises placing such an article to be protected, as anode in an acid electrolyte having a pH value above 2.5, but not substantially above 3.95, and such electrolyte being incapable of chemically attacking metallic magnesium, and said electrolyte consisting essentially of water containing a soluble manganese compound of chromic acid, said electrolyte also containing a small amount of at least one substance containing the anion of a mineral acid which mineral acid would in higher concentration be capable of chemically attacking magnesium, such acid being selected from the group consisting of sulphuric acid, nitric acid and phosphoric acid, the amount of such mineral acid ion being not more than 0.1% of sulphate ions, not more than 0.5% of nitrate ions, not more than 0.2% of phosphate ions, and placing a cathode in said electrolyte, but out of physical contact with said anode, such cathode being an electrically conductive material more noble than magnesium, electrically connecting said anode and said cathode outside said bath, the electrode

potential of the magnesium electrode in said electrolyte relatively to the hydrogen electrode being not over 1.1 volts, continuing the flow of said current until a protective film of substantial thickness has been formed on said anode.

2. A process for protecting, by galvanic action, an article made of metal consisting mainly of magnesium, wherein the article to be protected forms an anode in a galvanic cell, and the cathode is a more noble electrically conductive material, and the electrolyte in said cell is acid in reaction and consists essentially of an aqueous solution of a manganese compound of chromic acid as by far its largest dissolved component, also containing a substantial but very small amount of the anion of sulphuric acid, namely not more than 0.1% of  $\text{SO}_4^{2-}$  radical, the potential at said magnesium anode in said electrolyte relatively to the hydrogen electrode being lower than 1.1 volts, and the pH of the electrolyte being higher than 2.5 but not above 3.95, and said electrolyte being free of other substances which would affect the pH and the electrode potential of said magnesium anode.

3. A process as covered in claim 1, in which the cathode is carbon.

4. A process of providing a protective coating upon a metallic article composed substantially entirely of magnesium and magnesium base alloy, by galvanic action, which comprises placing such an article to be protected, as anode in an acid electrolyte having a pH value above 2.5, but not substantially above 3.95, and such electrolyte being incapable of chemically attacking metallic magnesium, and said electrolyte consisting essentially of water containing a soluble manganese compound of chromic acid, said electrolyte also containing a small amount but not over 0.1% of a substance containing  $\text{SO}_4$  ions, and placing a cathode in said electrolyte, but out of physical contact with said anode, such cathode being an electrically conductive material more noble than magnesium, electrically connecting said anode and said cathode outside said bath, the electrode potential of the magnesium electrode in said electrolyte relatively to the hydrogen electrode being not over 1.1 volts, continuing the flow of said current until a protective film of substantial thickness has been formed on said anode.

5. A process of providing a protective coating upon a metallic article composed substantially entirely of magnesium and magnesium base alloy, by galvanic action, which comprises placing such an article to be protected, as anode in an acid electrolyte having a pH value above 2.5, but not substantially above 3.95, and such electrolyte being incapable of chemically attacking metallic magnesium, and said electrolyte consisting essentially of water containing a soluble manganese compound of chromic acid, said electrolyte also containing a small amount, but not over 0.2% of a compound containing  $\text{PO}_4$  ions, and placing a cathode in said electrolyte, but out of physical contact with said anode, such cathode being an electrically conductive material more noble than magnesium, electrically connecting said anode and said cathode outside said bath, the electrode potential of the magnesium electrode in said electrolyte relatively to the hydrogen electrode being not over 1.1 volts, continuing the flow of said current until a protective film of substantial thickness has been formed on said anode.

6. A process of providing a protective coating upon a metallic article composed substantially

entirely of magnesium and magnesium base alloy, by galvanic action, which comprises placing such an article to be protected, as anode in an acid electrolyte having a pH value above 2.5, but not substantially above 3.95, and such electrolyte being incapable of chemically attacking metallic magnesium, and said electrolyte consisting essentially of water containing a soluble manganese compound of chromic acid, said electrolyte also containing a small amount but not over 0.5% of 10 a compound containing  $\text{NO}_3^-$  ions, and placing a cathode in said electrolyte, but out of physical contact with said anode, such cathode being an electrically conductive material more noble than magnesium, electrically connecting said anode and said cathode outside said bath, the electrode potential of the magnesium electrode in said electrolyte relatively to the hydrogen electrode being not over 1.1 volts, continuing the flow of 20 said current until a protective film of substantial thickness has been formed on said anode.

HERBERT MANFRED FREUD.

#### REFERENCES CITED

The following references are of record in the 25 file of this patent:

#### UNITED STATES PATENTS

| Number    | Name          | Date          |
|-----------|---------------|---------------|
| 1,838,273 | McBride       | Dec. 29, 1931 |
| 2,052,962 | Booe          | Sept. 1, 1936 |
| 2,206,028 | Buzzard       | July 2, 1940  |
| 2,224,528 | Sutton et al. | Dec. 10, 1940 |
| 2,356,575 | Frasch        | Aug. 22, 1944 |
| 2,463,483 | Frasch        | Mar. 1, 1949  |

#### FOREIGN PATENTS

| Number  | Country       | Date          |
|---------|---------------|---------------|
| 515,648 | Great Britain | Dec. 11, 1939 |
| 702,266 | France        | Apr. 3, 1931  |
| 471,053 | Germany       | Jan. 17, 1929 |

#### OTHER REFERENCES

Alien Property Custodian publication 297,191 of May 18, 1943.

"Metaux et corrosion," vol. 14 (1939), pages 87 through 91.

"Transactions of The Electrochemical Society," vol. 90 (1946), pages 503 through 507.